

Aug. 28, 1956

H. L. HARVEY

2,760,313

ABRASIVE WHEEL

Filed May 12, 1955



FIG. 3

## 1

2,760,313

## ABRASIVE WHEEL

Howard L. Harvey, Haddonfield, N. J., assignor to American Viscose Corporation, Philadelphia, Pa., a corporation of Delaware

Application May 12, 1955, Serial No. 507,786

11 Claims. (Cl. 51—209)

This invention relates to abrasive wheels and discs and a method of making such articles and, more particularly, to reinforced abrasive wheels and discs.

The present application is a continuation in part of my abandoned application, Serial No. 498,586, filed April 1, 1955.

Abrasive wheels and discs have been produced having a textile fabric reinforcement on one or both sides of the wheel or disc bonded to the body which consists of a molded mass of a binding material and the abrasive particles with or without additional strengthening materials and fillers, such as fibers and chopped rag. Because of the inherent nature of knitted and woven textile fabrics, the strength of the molded wheel or disc varied in different radial directions. A further disadvantage in wheels and discs of this type is that upon wearing of the grinding edge, the woven fabrics often leave a ragged edge.

The principal purpose of the present invention is to provide a grinding wheel or disc which has a substantially uniform strength in all radial directions.

Another purpose of the present invention is to provide a grinding wheel which will continuously present a smooth grinding surface as the wheel becomes worn.

A still further object of the invention is to provide a grinding disc having a reinforced construction of sufficient strength to prevent parts of the disc from breaking off even when the grinding face is fractured.

Other objects and advantages of this invention will become apparent from the following description and claims.

In the drawings:

Figure 1 is a transverse section of a grinding disc constructed in accordance with the present invention; and

Figure 2 is a back view of the disc of Figure 1 with the structure broken away and the spiral element exaggerated to more clearly illustrate its construction.

Figure 3 is a fragmentary detail of a grinding disc constructed in accordance with the present invention showing how the backing paper and the cord retain any pieces of the grinding face which may become fractured; and

Figure 4 is an enlarged sectional detail as seen at IV—IV of Figure 3.

The present invention is a continuation-in-part of United States patent application 498,586, filed on April 1, 1955, and contemplates an abrasive wheel or disc reinforced with a spirally laid cord and a long fibered paper which are bonded together, as by stitching, and bonded to the abrasive material.

Referring more particularly to the drawings, the present grinding disc has a centrally perforated backing sheet or disc 1 of a latex impregnated long fibered paper. This paper is rigidly adhered or stitched to a spiral layer of cord 2 which is preferably laid on the paper in close convolutions. The abrasive grinding face 3 is likewise bonded to the layer of cord and comprises suitable grits in a binder. The disc is provided with the customary off-

## 2

set hub 4 having a bore 5 for mounting on the grinder spindle. The elements of the wheel when finished form a unitary tough structure which cannot be fractured into small pieces under any conditions of use or even abuse.

5 The long fibered paper is preferably a paper formed of fibers having the length of from four to seven millimeters and the fibers have diameters of from seventeen to twenty-five microns. The paper is preferably formed without sizing and is impregnated with latex, either a synthetic or natural elastomeric material dispersion. The paper may be formed of hemp or abaca fibers and may contain from about 100% to about 165% by weight of the latex. Paper, such as described in Patent No. 2,541,763 has been found to be very satisfactory for the purposes of this invention. Silicone rubbers may also be used to impregnate the long fibered paper.

The spirally laid cord may be formed of any desired fibrous strand, such as cotton, rayon, nylon, or other synthetic fibers such as "Dacron," "Acrilan," "Orlon" and the like. The size or diameter of the cord or strand may be selected to provide the desired reinforcement. For example, it may be varied in diameter depending upon the thickness of the grinding wheel or disc and the speed at which the grinding disc will be operated. The 15 cord may be impregnated with or treated with a thermosetting resin, as for example urea-formaldehyde, melamine-formaldehyde, and phenol-formaldehyde in the thermoplastic state and containing a latent curing catalyst, either before or after it is disposed in the spiral position.

The abrading element 3 is of any desired composition. The active abrasive material may consist of any desired abrasive grit or grain, such as aluminum oxide, silicone carbide, boron carbide, diamonds, emery and the like. 20 The size of the abrasive particles and the particle size distribution may vary and will be selected for the particular use of the particular grinding wheel. For example, if the wheel is to be adapted to coarse grinding, the particles selected will be relatively large whereas for finished grinding or polishing, the particles will be fine.

The bonding material selected will likewise be based upon the intended use of the specific wheel or disc. The so-called resinoid type of binders find extensive use in this 25 art and may be employed in the products of this invention. These binders include various grades of phenol-formaldehyde resins, urea-formaldehyde resins, melamine-formaldehyde resins and other amino triazine resins. The abrasive element may be formed in any desired manner as

30 by mixing the abrasive grits or grains with the powdered resinoid or the abrasive grits may be first coated with the resinoid and then mixed with additional quantities of the bonding material. The abrasive grits may be coated with a specific bonding material and the bulk of the bonding material may consist of a different specific material. For example, the abrasive grits may be wet with a phenolic condensation product and the coated grits then mixed with an amino triazine aldehyde condensation product and the mixture subsequently molded.

35 Fillers or substances and materials to strengthen or improve the impact resistance of the abrading element may be incorporated in the mix prior to molding to shape, for example, fibers of various lengths or chopped rag formed of either natural or synthetic fibers may be incorporated in the mixture to improve the impact resistance and flexural strength of the abrading element. These types of filler materials may be impregnated with a resinoid material to insure a thorough bonding between the constituents of the abrading element. Other fillers, such as clay, asbestos fiber, mica or other materials commonly used in abrading elements may also be present.

It is apparent that the specific constituents and the relative proportions of the various constituents will be determined by the intended use of any specific grinding wheel. The composition of the abrading element does not form a part of the present invention. However, the present invention is applicable to any and all abrading wheels and discs wherein the abrading element contains a bonding material which may be bonded to the spirally laid cord reinforcement.

In forming the grinding wheels or discs in accordance with this invention, the impregnated long fibered paper disc is held at its center opening in a manner so as to permit it to be moved concomitantly in rotary and side-wise directions. A cord or strand 2 may be adhesively secured to the paper disc 1 but in the preferred form 10 of the invention the cord 2 is laid on the paper disc 1 in a spiral manner and held in place by a light thread stitched as seen at 6 in Fig. 2. For the sake of clarity and simplicity, only a small portion of the stitching has been illustrated on the drawing, it being understood that 20 all convolutions of the cord are secured to the paper disc by stitching. As described above the cord or strand 2 is impregnated with a thermosetting resin, for example, a rayon cord such as conventionally employed in the manufacture of tire casings may be impregnated with a phenolic resin and laid on the paper disc without converting the resin to its thermoset condition. By securing the reinforcing cord 2 to the paper disc as set forth above, the spiral cord formation and the paper disc itself are better able to retain their original and intended shapes 30 during molding. The paper disc, with the cord secured thereto, is placed in the mold and the abrading material, either in the form of a powder or granular mix or in the form of a preformed disc containing the thermosetting resin in a thermoplastic condition, is then placed over 35 the spirally laid cord. The mold is then closed and the laminated body subjected to the required pressures and temperatures whereby the elements become bonded together to form a unitary body. The wheel or disc which is formed may be employed as a grinding wheel or a 40 grinding disc.

During the molding operation, the stitching thread holding the spiral cord formation on the paper disc 1 is subjected to high temperature and pressures of approximately 3,000 pounds per square inch and therefore have a tendency to break. However, once the molding operation is underway, the stitching has already served its purpose and the broken threads in no way impair the 45 desired qualities of the finished product.

Where the product is to be utilized as a grinding wheel, a disc of any desired material may be placed in the mold over the abrading material prior to the molding operation. This surfacing material may consist of a woven textile fabric formed of organic or inorganic fibers or it may be formed of a non-woven fibrous sheet, such as 50 paper or it may consist of another spiral cord laid and stitched to a disc of long fibered paper.

Grinding wheels, formed as herein described, have a uniform strength in all radial directions. It is well known that textile fabrics impregnated with phenolic resins and used as reinforcing elements in grinding wheels are exceedingly brittle. If a grinding wheel having such reinforcement is accidentally subjected to a blow, the reinforcing element readily cracks and if the grinding wheel is operating at a high speed, the wheel will fly apart. Wheels of the present invention, although they have been subjected to a blow sufficient to crack the abrading element through its entire thickness, have been operated 55 at speeds far in excess of the normal operating speed for

the wheel without flying apart. Comparable grinding wheels having nylon and glass fiber textile reinforcing elements or discs when operated under the same conditions have generally been found to fly apart upon fracture of the abrading element.

It has also been found that as the grinding surface becomes worn down, the peripheral edge of the spirally laid cord and the paper become worn away without leaving a ragged edge as is so common in the case of the usual textile reinforcing elements.

In forming the grinding wheel as described above and utilizing pressures exceeding about 3000 pounds per square inch, the reinforcing element appears to be a unitary body wherein the paper disc and spirally laid cord are so thoroughly bonded together that it is difficult to distinguish between the two elements. The strength of the wheel and the characteristic of the fractured wheel of being capable of withstanding excessive speeds is not obtainable by the use of either a spirally laid cord or a long fibered paper. It is only by the combination of the two that these characteristics are obtained.

I claim:

1. In a grinding wheel a reinforcing element comprising a long fibered paper and a spirally laid cord, the paper and the cord being combined into an integral body.
2. A reinforcing element as defined in claim 1 wherein the paper is formed of abaca fibers.
3. A reinforcing element as defined in claim 1 wherein the cord is formed of rayon.
4. A reinforcing element as defined in claim 1 wherein the paper is formed of abaca fibers and is impregnated with a latex and the cord is formed of rayon impregnated with a phenolic condensation product.
5. A construction as defined in claim 1 wherein said paper and cord are combined by stitching.
6. The method of forming a grinding wheel which comprises sewing a spirally laid cord to a long fibered paper, positioning the combined paper and cord in a mold, placing an abrading composition over the spirally laid cord and applying heat and pressure to bond the paper, cord and abrasive composition together to form a unitary body.
7. A non-fracturable grinding wheel having a backing sheet of long fibered latex impregnated paper, a spiral cord to which said backing sheet is bonded, and a grinding face of abrasive grits bonded to said cord.
8. A grinding wheel in accordance with claim 7 in which the long fibers are abaca.
9. A grinding wheel comprising an abrading disc having on at least one of its sides a reinforcing element comprising a spirally laid cord bonded to the abrasive element and a long fibered paper bonded to the spirally laid cord.
10. A grinding wheel in accordance with claim 9 in which the paper and cord are bonded by stitching.
11. The method of forming a grinding wheel which comprises positioning a long fibered paper in a mold, disposing spirally laid cord over the paper in the mold, placing an abrading composition over the spirally laid cord and applying heat and pressure to bond the paper, cord and abrasive composition together to form a unitary body.

References Cited in the file of this patent

UNITED STATES PATENTS

2,260,941 Hendrickson Oct. 28, 1941